

# United States Patent [19]

Sawyer et al.

[11] 3,768,738

[45] Oct. 30, 1973

[54] FLOTATION OF ARSENIC MINERALS  
FROM BORATE ORES

[75] Inventors: Dwight L. Sawyer, Boron; Martin  
Wilson, Anaheim, both of Calif.

[73] Assignee: United States Borox & Chemical  
Corporation, Los Angeles, Calif.

[22] Filed: Oct. 21, 1971

[21] Appl. No.: 191,536

[52] U.S. Cl..... 241/24, 209/11, 209/166,  
209/164

[51] Int. Cl..... B03b 1/02

[58] Field of Search..... 209/166, 167, 11,  
209/3, 17; 241/20, 24

## [56] References Cited

### UNITED STATES PATENTS

835,143 11/1906 Sulman ..... 209/166

|           |         |                  |           |
|-----------|---------|------------------|-----------|
| 1,208,334 | 12/1916 | Lavers .....     | 209/166   |
| 2,184,558 | 12/1939 | Malozemoff ..... | 209/166 X |
| 2,257,710 | 9/1941  | Archibald .....  | 209/166   |
| 2,317,413 | 4/1943  | Shelton .....    | 209/166   |
| 2,741,364 | 4/1956  | Wilson .....     | 209/166 X |

### FOREIGN PATENTS OR APPLICATIONS

|           |         |               |         |
|-----------|---------|---------------|---------|
| 100,223   | 11/1940 | Sweden.....   | 209/166 |
| 602,686   | 12/1925 | France .....  | 209/166 |
| 749,467   | 5/1944  | Germany ..... | 209/166 |
| 1,137,115 | 1/1957  | France .....  | 209/166 |

Primary Examiner—Robert Halper

Attorney—James R. Thornton

### [57] ABSTRACT

Arsenic minerals, such as realgar, may be removed by flotation from hot slurries of borate ores, such as ulexite, colemanite and tincal with or without the aid of a flotation reagent.

10 Claims, No Drawings

### FLOTATION OF ARSENIC MINERALS FROM BORATE ORES

In accordance with the precepts of the invention, realgar,  $As_4S_4$  or  $As_2S_2$ , the predominant arsenic mineral in soluble borax ore, such as tincal, is removed by flotation of a hot approximately saturated slurry, preferably at least 75° C., although such removal cannot easily be obtained if the slurry is at room temperature. A pH adjustment is not required because flotation occurs readily at the natural pH of about 9.2. The process may be carried out without the use of a flotation reagent, although if desired, one may be used to enhance the ease of flotation. This process makes it possible to remove between about 80 percent to 98 percent of the contained arsenic by means of a flotation process, wherein oftentimes only a single step may be necessary. This is unexpected in view of the slime forming clay content of such ore. Flotation of realgar in saturated borax solutions at room temperature is sluggish and incomplete.

Similarly, it has been found that the same flotation technique may be applied with other borate ores, such as ulexite and colemanite. Ulexite is a natural hydrated borate of sodium and calcium,  $NaCaB_5O_7 \cdot 8H_2O$ . Colemanite is a natural hydrated calcium borate  $Ca_2B_6O_{11} \cdot 5H_2O$ . However, the solubility of these ores are considerably less in water than tincal.

It has also been discovered that when applying the method of the present invention to a borax containing ore such a tincal, the considerable amount of strong borax liquor present in the floated realgar may be recovered to make the process more economical. Filtration of the concentrate is difficult because of the clay slimes present. The desired further recovery may be accomplished by refloating the concentrate after dilution with weak liquor. The cleaner concentrate slurry, containing mainly weak liquor, may be discarded and the cleaner tailings slurry is returned to the ore dissolver.

In carrying out the invention, the ore slurry is prepared by crushing the ore to at least minus 20 mesh, preferably minus 50 mesh and then heating with water, or by heating the coarse ore with water and passing the solution through a 50 mesh screen.

Commercial flotation cells may be used as rougher cells and as cleaner cells. For relatively small scale operations, the well known Denver Lab cells, manufactured by Denver Equipment Company, were employed in the examples set forth below. The cells may be operated in series to improve the efficiency of the process.

zone at the uppermost portion of the cell where cell action is quiet. Applicable froth flotation cells are described in KIrk-Othmer Encyclopedia of Chemical Technology, Second Edition (1966), Volume 9, pages 391 and 392.

Short hydrocarbon chain ( $C_2$  to  $C_5$ ) xanthates or low viscosity mineral oils, such as kerosene, diesel oil and Bunker oil, may be used as flotation reagents (collectors and frothers), if desired. These reagents are then used in the manner well known in the art.

The water insolubles in the rougher tailings slurry are flocculated. After settling in a thickener, the hot overflow brines are sent to a crystallizer.

15

### EXAMPLES I-VI

An approximately saturated borax slurry was prepared by crushing 150 g. of soluble tincal to minus 50 mesh, slurring with 250 ml. of water, and heating the mixture to 95° to 100° C. When flotation agents were employed, as in Examples I-V, they were added to the hot slurry. After thirty seconds conditioning, the slurry (at 95° C.) was transferred to a 100 g. Denver Lab cell where air froth flotation was maintained for 2.5 minutes. The test data are set forth in the following Table I.

TABLE I

| Example | Tincal ore         |                                         | Kind         | Lb./ton | Arsenic distribution, percent |       |
|---------|--------------------|-----------------------------------------|--------------|---------|-------------------------------|-------|
|         | Insoluble, percent | As <sub>2</sub> O <sub>3</sub> , p.p.m. |              |         | Conc.                         | Tails |
| I       | 3                  | 8,200                                   | Ethyxanthate | 0.5     | 98.2                          | 1.8   |
| II      | 14                 | 3,800                                   | do           | 0.25    | 86.9                          | 13.1  |
| III     | 14                 | 3,800                                   | do           | 0.125   | 89.2                          | 10.8  |
| IV      | 20                 | 1,700                                   | Kerosene     | 0.5     | 79.8                          | 20.2  |
| V       | 14                 | 3,800                                   | do           | 0.25    | 86.9                          | 13.1  |
| VI      | 14                 | 3,800                                   | None         | -----   | 85.8                          | 14.2  |

### EXAMPLES VII-IX

Examples VII-IX show the influence of water insolubles and orpiment ( $As_2S_3$ ) on the process. The ore used for Example IX contained some orpiment and turned yellow during crushing. The ore for Example VII was crushed to minus 20 mesh while those for Examples VII and IX were crushed to minus 50 mesh. Except as noted, the flotation were carried out as in conjunction with Examples I-V, that is, in the presence of flotation reagents. As would be expected with an increase in insolubles, the tails are increased.

TABLE II

| Example | Ore analysis       |                                         | As <sub>2</sub> O <sub>3</sub> after flotation, p.p.m. | Reagent      | As distribution |         |         |
|---------|--------------------|-----------------------------------------|--------------------------------------------------------|--------------|-----------------|---------|---------|
|         | Insoluble, percent | As <sub>2</sub> O <sub>3</sub> , p.p.m. |                                                        |              | Kind            | Lb./ton | Concen- |
| VII     | 2-3                | 8,200                                   | 151                                                    | Ethyxanthate | 0.5             | 98.2    | -----   |
| VIII    | 20                 | 1,700                                   | 340                                                    | Kerosene     | 0.5             | 79.8    | -----   |
| IX      | 5-7                | 3,200                                   | 568                                                    | do           | 0.5             | 82.3    | -----   |

In the Denver cell, the slurry flows into the machine by gravity through the feed pipe, dropping the slurry directly on the top of the rotating impeller below a stationary hood. This is the mixing and aeration zone where air is drawn in by positive suction down a stand-pipe into the heart of the cell. Zone 2 is the separation zone where the arsenic-laden air bubbles separate from the borate solution or slurry. Zone 3 is the concentrate

### EXAMPLES X - XIV

The special influence of flotation reagents is illustrated by Examples X-XIV. The ore contained about 14% water-insolubles and about 3,800 ppm. As<sub>2</sub>O<sub>3</sub>. The slurry particles were less than 20 mesh and were processed as before.

3  
TABLE III

| Example | Kind          | Lb/Ton | Concen-<br>trate | Tails | 5 |
|---------|---------------|--------|------------------|-------|---|
| X       | Ethylxanthate | 0.5    | 88.3%            | 11.7% |   |
| XI      | "             | 0.25   | 88.9             | 13.1  |   |
| XII     | "             | 0.125  | 89.2             | 10.8  |   |
| XIII    | None          | —      | 85.8             | 14.2  |   |
| XIV     | Kerosene      | 0.25   | 86.9             | 13.1  |   |

It will be seen from the above that more arsenic is floated from the cell when a flotation agent is employed.

#### EXAMPLES XV – XVII

In each of the following examples, a 100 g. Denver flotation cell was charged with 50 g. of minus 100 mesh ulexite ore which was slurried with 40 ml. of water. The temperature of the slurry was as indicated in Table IV. The pH was 9.0 when cold and 9.2 when hot. Additional water was added, hot in the case of XV and XVI examples. Air was introduced to produce a good froth. Each flotation step, in conjunction with each example, was run 9.0 2.5 minutes.

The first flotation gave a first tail and an arsenic concentrate. The concentrate was refloated to give a second tail and the final concentrate. In examples XV and XVII, no flotation reagents were included while in example XVI, two drops of kerosene was included. The temperature during the flotation steps was as indicated in Table IV.

It will be seen that arsenic recovery is higher in the final concentrate when a flotation reagent is employed. In example XVII, the arsenic recovery in the final concentrate is only 67.3 percent of the total. However, it will be also seen that the temperature of the slurry during the flotation steps was only between 27° to 33° C., clearly demonstrating that the higher temperatures produce admirably better results.

TABLE IV

Starting Ore — Ulexite Containing 4080 ppm. As  
Example XV Flotation Reagent — None

|                   | Temperature (°C.) | Start | Finish |       |
|-------------------|-------------------|-------|--------|-------|
|                   | First Flotation   | 90    | 84     |       |
|                   | Second Flotation  | 93    | 85     |       |
|                   |                   |       |        | % of  |
|                   |                   |       |        | Total |
| First Tail        | 31.4              | 26    | 0.4    | As    |
| Second Tail       | 5.9               | 1520  | 4.3    |       |
| Final Concentrate | 2.6               | 76800 | 95.3   |       |
| Total             | 39.9              |       |        |       |

Example XVI Flotation Reagent — Kerosene (2 drops)

|                   | Temperature (°C.) | Start  | Finish |       |
|-------------------|-------------------|--------|--------|-------|
|                   | First Flotation   | 92     | 86     |       |
|                   | Second Flotation  | 95     | 80     |       |
|                   |                   |        |        | % of  |
|                   |                   |        |        | Total |
| First Tail        | 33.2              | 80     | 1.3    | As    |
| Second Tail       | 5.2               | 68     | .2     |       |
| Final Concentrate | 2.5               | 80,000 | 98.5   |       |
| Total             | 40.9              |        |        |       |

4  
Example XVII Flotation Reagent — None

|                   | Temperature (°C.) | Start | Finish |
|-------------------|-------------------|-------|--------|
|                   | First Flotation   | 27    | 30     |
|                   | Second Flotation  | 29    | 33     |
|                   |                   |       | % of   |
|                   |                   |       | Total  |
| First Tail        | 28.1              | 1080  | 19.1   |
| Second Tail       | 9.3               | 2320  | 13.6   |
| Final Concentrate | 4.9               | 21800 | 67.3   |
| Total             | 42.3              |       |        |

As stated in the above, when operating with a soluble ore such as tincal there is considerable loss of soluble borate in the first or rough concentrate. While the examples in the above pertaining to ulexite incorporate a second flotation, the same procedure is suggested with regard to tincal in order to recover the soluble borate which may be lost in the rougher concentrate.

Although the examples described in the above were carried out in a Denver Lab cell having a capacity of 100 ml., in commercial operation cells having a capacity of 2 to 100 cubic feet, preferably from 40 to 100 cubic feet, would be used. These larger cells will give a lower strong borax retention in the rougher concentrate and a lower arsenic transfer to the cleaner tailings, thereby improving the efficiency of the process.

It will be apparent that many changes and modifications may be made in the process described herein without departing from the spirit and scope of the invention. It is therefore apparent that the foregoing description of by way of illustration of the invention and not by way of limitation.

What is claimed is:

1. The method of removing arsenic sulfide minerals from hydrated sodium and calcium borate containing ores comprising the steps of forming an aqueous slurry of said ore at a temperature of from about 75° to about 100° C., and subjecting said hot slurry to froth flotation and then separating the tailings from the floated materials which will contain a concentrate of said minerals.
2. The method of claim 1 wherein said slurry is conditioned with a flotation reagent selected from the group consisting of alkyl xanthates having two to five carbon atoms, kerosene, diesel oil and bunker oil prior to the flotation step.
3. The method of claim 1 wherein the mineral is realgar.
4. The method of claim 1 wherein the ore is tincal.
5. The method of claim 1 wherein the ore is ulexite.
6. The method of claim 1 wherein the ore is colemanite.
7. The method of claim 1 wherein the process is conducted at the natural pH of the ore of about 9.
8. The method of claim 1 wherein said ore is crushed to at least minus 20 mesh prior to forming said aqueous slurry.
9. The method of claim 1 wherein said ore is crushed to at least minus 50 mesh prior to forming said aqueous slurry.
10. The method of claim 1 wherein said aqueous slurry is passed through a 50 mesh screen prior to froth flotation.

\* \* \* \* \*

UNITED STATES PATENT OFFICE  
CERTIFICATE OF CORRECTION

Patent No. 3,768,738 Dated October 30, 1973

Inventor(s) Dwight L. Sawyer and Martin Wilson

It is certified that error appears in the above-identified patent and that said Letters Patent are hereby corrected as shown below:

In Column 2, line 3 delete "KIrk" and add --Kirk--;

In Column 2, line 44 delete "VII" and add --VIII--;

In Column 2, TABLE II under the heading "Tails", line 57  
add --percent--;

In Column 2, line 58 delete "-----" and add --1.8--;  
line 59 delete "-----" and add --20.2--;  
line 60 delete "-----" and add --17.7--;

In Column 3, line 22 delete "9.0" and add --for--.

Signed and sealed this 16th day of April 1974.

(SEAL)  
Attest:

EDWARD M.FLETCHER, JR.  
Attesting Officer

C. MARSHALL DANN  
Commissioner of Patents